

G. R. GEHRANDT.  
PROCESS OF SMELTING AND PURIFYING IRON.  
APPLICATION FILED JUNE 14, 1913.  
1,110,540.

Patented Sept. 15, 1914



WITNESSES:

*Aug. Winter*  
*Henry Fain*

INVENTOR

*Gustave R. Gehrandt*

BY *Robt. Steff*  
*and E. A. Tolson*

ATTORNEYS

# UNITED STATES PATENT OFFICE.

GUSTAVE R. GEHRANDT, OF CHICAGO, ILLINOIS.

## PROCESS OF SMELTING AND PURIFYING IRON.

1,110,540.

Specification of Letters Patent. Patented Sept. 15, 1914.

Application filed June 14, 1913. Serial No. 773,593.

To all whom it may concern:

Be it known that I, GUSTAVE R. GEHRANDT, a subject of the Emperor of Germany, residing at Chicago, Illinois, have invented certain new and useful Improvements in Process of Smelting and Purifying Iron, of which the following is a specification.

The essential object of this invention is to produce a pig iron which is very much purer than any ordinary pig now obtained in commercial quantities.

By the use of the herein-described invention, the operator simultaneously, and in the same furnace, both smelts the ore (reducing the same to iron) and purifies the iron yielded by the smelting process.

The pig iron produced by this invention may either be subjected to further treatment, or may be used just as it comes from the furnace, for by employing this invention it is possible to control, within certain limits, the chemical composition of the pig.

Although the process is described with reference to its performance by one particular apparatus or furnace which is adapted to perform the process, it should be understood that the invention resides in the process and not in any particular furnace or apparatus and that other forms of apparatus may be employed for the performance of the process which forms the subject-matter of this application.

In the drawings, the single figure is a vertical section of a blast furnace adapted to practise the invention, and said furnace comprises the stack 1, bosh 2, and hearth 3. The bustle pipe 4 carries an air-blast and to said pipe there may be applied such of the appliances for controlling the pressure, temperature, and volume of the air as the judgment of the operator may determine.

A second bustle pipe 5 is provided, and the twyters 6 and 7 extend from pipes 4 and 5, respectively, to the hearth. Twyters 6 are horizontally disposed and twyters 7 are oblique, being arranged with their discharge ends uppermost, so as to direct the streams of air upwardly at an angle oblique to the level of the molten iron. Two perforations 8 and 9 are provided, said perforations being called cinder-notches by some furnace-workers, and slag-holes by others, cinder-notches 8 being located just beneath the twyters 6 and above twyters 7, and cinder-

notch 9 being just below twyters 7. The iron-notch 10 is arranged in the usual way near the bottom of the hearth, and all of the notches 8, 9, and 10 are adapted to be plugged by fire clay in the usual manner. Preferably the obliquely-disposed twyters 7 are so arranged that their axial lines produced all meet approximately at the axial line of the furnace. It is well-known that in the operation of the ordinary blast-furnace, the stack is charged with a mix of ore, flux, coke (or other fuel), and such other articles as are required, and that an air-blast is forced into the furnace through the twyters, which are usually arranged above the highest level which the molten mass of metal and slag can attain. The resultant product is the commercial pig iron, pig being chemically an alloy of iron and sundry elements and compounds thereof, such as carbon, silicon, manganese, phosphorus, sulfur, &c., and in the arts it is frequently necessary to free the iron from some or all of its impurities, both metallic and non-metallic.

Many ways of purifying iron or of converting same into steel have been employed, but heretofore all such processes have necessitated the removal of the pig iron from the blast-furnace to a different apparatus, such as a converter, where a separate and distinct step of the process of making the ultimate product, whatever it may be, is performed; whereas in this invention the iron is purified, or partly so, in the same furnace in which the ore is smelted, and thus the operator dispenses with the necessity of one handling of the metal, and is enabled to produce a pig iron much purer than any heretofore known and an iron the chemical composition of which can be regulated and determined within reasonable limits. Otherwise stated, the purifying process and the smelting process proceed simultaneously, and in the same furnace, and one apparatus produces a finished product for the production of which two apparatuses were formerly required.

In the operation of the furnace the same is charged with the usual mix, and started just as any ordinary blast-furnace. The slag at first is drawn through cinder-notch 9, but soon enough iron will accumulate for the level of the molten liquid to rise to a point where the slag can be drawn through 112

cinder-notch 8, cinder-notch 9 being plugged in due season. The molten iron thus rises over the mouths of the twyers 7, and, hence, the air-blast from pipe 5 will pierce the metal and oxidize the impurities of the molten iron. By regulating the quantity, temperature, and pressure of the blast it is possible to determine, within reasonable limits, the chemical constituency of the pig iron. The blast from the upper twyers 6 will not pierce the metal, but will pass through the mix in the bosh 2 and stack 1 in the usual manner.

From one point of view, the twyers 6 are only emergency twyers, for ordinarily the oblique twyers will deliver enough air for the entire process, including both the smelting and the decarburizing, notwithstanding the fact that much of the oxygen delivered thereby is consumed and utilized when passing through the iron; but it is better and safer to provide the two sets of twyers than to rely upon one set alone, for at times when the flow of air through twyers 7 is checked, possibly not enough air would be delivered to furnish the oxygen required for the smelting process. With two sets of twyers, one can be used for the smelting and the other for the oxidizing, and each set controlled at will, without any fear that the smelting will be impaired merely because only a short air-supply is required for the oxidization.

It is to be observed that this invention is not a "direct" process of producing steel itself from iron ore, for while the final product of this invention is an iron which is freed, in whole or in part, from carbon, silicon, and other metallic and non-metallic impurities, the molten metal escaping from the iron notch 10 still requires further treatment to convert it into steel. The pig iron produced by this invention is, however, a refined or purified pig, and is a product which can be used for countless purposes for which ordinary commercial pig is unsuitable, unless it be further treated by some process of purification or refining.

In the practice of the invention, the molten iron in the hearth 3 is allowed to accumulate until it stands at a higher level than the mouths of the twyers 7. There will, of course, be a layer of slag on top of the mass of molten iron, which slag can be drawn off from time to time through the cinder-notch 8. The air-blast from the twyers 7 will enter the body of molten iron near its outer and upper edge, and the stream of air will enter and pierce the molten iron and slag following oblique paths, the angle of which depends upon the angle of inclination of the twyers 7. The blast from the twyers 6 will enter the furnace, following paths which are approximately horizontal at the mouths of the twyers 6. It

will be obvious, therefore, that the mass of molten metal which collects in the hearth is covered by what may conveniently be termed an air umbrella; that is to say, the various streams from the obliquely-disposed twyers 7 will tend to pierce the body of molten iron near the upper level and to pierce the slag, passing through both metal and slag at an oblique angle, and streams from twyers 7 will center at approximately the median line of the stack. Some of the oxygen of the air which enters through the oblique twyers 7 will be exhausted in passing through the molten iron and slag, but an additional volume of oxygen will be supplied by the air from twyers 6. Because of the forming of this air umbrella, every particle of smelted ore dropping from the stack or bosh into the hearth must pass through the heated air before reaching the hearth, and every such particle of smelted ore is, accordingly, partly purified before it even reaches the hearth.

In a blast furnace of ordinary size, it is customary to collect approximately 150 tons of molten metal in the hearth, and should the air blast enter this body of metal near the bottom, it is certain that the agitation thus caused would eventually rupture even the strongest furnace, whereas, in this invention by causing the stream of air to enter near the top of the body of molten metal, the agitation within the hearth is kept well within the limits of safety. Moreover, were the jets of air to enter near the bottom of the hearth, the air umbrella might not be formed and the partial purification which results from the action of the air umbrella upon the drops of freshly-smelted iron which pass through the air umbrella might not be secured.

If the streams of air were to enter the hearth at or near its bottom, much greater power would be required to cause the air-blast to pierce the metal, and it would be necessary to provide either more air-compressors or compressors of greater power in order to overcome the resistance and weight of the entire body of metal than are required where the streams of air enter near the top level of the molten metal. By arranging the twyers 7 near the top level of the molten metal, the air-blast which pierces the metal is not required to be under an abnormal or an excessive pressure; whereas, if the twyers 7 were to enter the hearth at or near its bottom, the pressure required to enable the air-blast to pierce the metal would be excessive.

Because of the fact that the air-blast from the twyers 7 pass obliquely through the metal, it follows that the agitation of the mass of molten metal is confined to a circular or annular space, and the metal or slag near the outer wall of the hearth is not violently agitated at any time; hence, it is not

a difficult matter to draw off the layer of slag. If the air-blast entered the bottom of the hearth, the agitation of the molten metal within the hearth would be such as to render it difficult to draw off the slag without simultaneously drawing off and wasting part of the iron; whereas, in this invention the streams of air from twyers 7 which pierce the metal pass therethrough at an oblique angle, leaving the surfaces of the metal or slag near the walls relatively smooth, thus permitting the slag to be drawn off when it reaches the proper height in the manner common to blast furnace practice.

15 It should be observed, finally, that to cause the stream of air to enter the mass of molten metal near the top level of the metal rather than at or near the bottom of the hearth does not interfere in any degree with 20 the efficacy of the purifying process. As is well known, a cubic foot of steel weighs about 490 pounds and a cubic foot of ordinary pig iron about 450 pounds, this difference in weight being due to the fact that the 25 impurities, such as carbon, silicon, phosphorus, sulfur, &c., are of lower specific gravity than iron itself. Since the lighter molten metal will tend to rise to the top while the heavier metal sinks to the bottom, 30 it is obvious that the stream from twyers 7 will cause a circulation of the molten metal within the hearth. As these streams pierce the molten metal and thus free that volume of metal through which said streams have 35 passed from some or all of its impurities, the specific gravity of the then purified metal is thereby increased and that metal through which said streams have passed is heavier after being freed of its impurities 40 than it is before being so freed. The heavier and purer metal will, of course, sink to the bottom, and as it does so, it is replaced by the lighter and more impure metal which will rise from the bottom to the top, and it 45 is evident, therefore, that to force the stream of air which pierce the metal within the hearth, suffice to purify the entire mass of molten metal.

I claim as my invention:

50 1. The herein described process of producing a purified iron which consists in smelting the ore, collecting the smelted ore in the hearth of the smelting furnace and in causing an air-blast to enter the smelted iron and 55 to enter and pierce the same at an angle

oblique to the level of the smelted iron, said air-blast being passed through the iron simultaneously as the supply of iron in the hearth is replenished by freshly smelted iron from above.

60

2. The herein described process of producing a purified iron which consists in smelting the ore, collecting the molten mass thus obtained in a receptacle beneath the ore, and in causing an air-blast to enter and 65 pierce said molten mass at a point adjacent the top level of said mass and to travel obliquely to the level of said mass, said air-blast being passed through the molten mass before the same is withdrawn from the receptacle.

70

3. The herein described process of producing a purified iron which consists in smelting the ore, collecting the reduced molten iron in the smelting apparatus, and 75 in causing an air-blast to enter the molten iron near the upper level of the body thereof, and in further causing said air-blast to pass through said iron while the same still remains in the receptacle within which it 80 has been collected.

76

4. The herein described process of producing a purified iron consisting in smelting the ore, collecting the reduced ore in the hearth of the smelting furnace, and in causing an air-blast to enter and pierce the iron at a point adjacent the upper level of the iron, said air-blast being passed through the iron in the hearth simultaneously as the supply of iron in the hearth is replenished by 85 freshly smelted iron from above.

80

5. The herein described process of producing a purified iron which consists in smelting the ore, collecting the reduced molten iron in the smelting apparatus, in 90 causing an air-blast to enter the molten iron near the upper level of the body thereof, in further causing said air-blast to pass through said molten iron while the same still remains in the receptacle within which 95 it has been collected, and in causing another air-blast to enter intermediate the upper level of the reduced molten iron and the body of the ore.

100

In testimony whereof I hereunto affix my 105 signature in the presence of two witnesses.

GUSTAVE R. GEHRANDT.

Witnesses:

ROBT. KLOPF,  
ELLIOTT R. GOLDSMITH.